

[54] **METHOD OF MANUFACTURING WIRES CONSISTING AT LEAST SUPERFICIALLY OF BORON AND WIRES OBTAINED BY SAID METHOD**

[75] Inventors: **Wubbe Vrieze, Otmar Schob**, both of Emmasingel, Eindhoven, Netherlands

[73] Assignee: **U.S. Philips Corporation**, New York, N.Y.

[22] Filed: **Oct. 18, 1971**

[21] Appl. No.: **190,378**

[30] **Foreign Application Priority Data**

Oct. 21, 1970 Netherlands ..... 7015375

[52] U.S. Cl..... **156/3, 156/2, 252/79.2**

[51] Int. Cl. .... **C23f 17/00**

[58] **Field of Search** ..... 156/2, 3; 252/79.2

[56] **References Cited**

UNITED STATES PATENTS

2,879,147 3/1959 Baker..... 156/24

3,446,682 5/1969 Wawner..... 156/3

*Primary Examiner*—Jacob H. Steinberg

*Attorney*—Frank R. Trifari

[57] **ABSTRACT**

To enhance the tensile strength, boron-coated tungsten wire may be etched with an etchant comprising phosphoric acid, nitric acid and water.

**3 Claims, No Drawings**

**METHOD OF MANUFACTURING WIRES  
CONSISTING AT LEAST SUPERFICIALLY OF  
BORON AND WIRES OBTAINED BY SAID  
METHOD**

The invention relates to a method of manufacturing wires which at least at their surface consists of boron, in which boron is deposited on a support and in which a part of the boron surface is subsequently etched off by means of an etchant comprising nitric acid.

Such a method is known, for example, from U.S. Pat. No. 3,446,682.

The purpose of etching off a part of the boron surface is to remove surface errors which have a detrimental influence on the mechanical properties of the wires and to enhance, *inter alia*, the tensile strength of the wires.

In "Boron" vol. 2, edition G.K. Gaule, pages 283 to 300 ("The effect of Chemical Polishing on the Strength and Fracture Characteristics of Amorphous Boron Filaments" by F.E. Wawner Jr.) it has been stated that optimum results can be achieved with mixtures of concentrated nitric acid and water in a volume ratio of 1:1. The etching rate is then approximately 2.5 micrometres per minute at a temperature of 100°C the etchant. Less satisfactory results are obtained with other ratios, with mixtures of sulphuric acid and nitric acid and with potassium periodate solutions. In practice, however, it was found that highly varying results may be obtained when using mixtures of concentrates nitric acid and water in a ratio of 1:1. In some wires the mean etching rate is more than approximately 2.5 micrometres per minute, particularly when etching takes place over a comparatively long period. In other wires hardly anything is etched off during exposure to the etchant.

This can only be explained when it is assumed that very pure crystallized boron is coated with an oxide layer protecting against attack by the etchant during etching with an etchant having an oxidising effect.

The etching rate is then especially determined by the density of the boron oxide layer, by the rate at which these oxides dissolve in the etchant and by the presence or absence of impurities.

An object of the present invention is to provide a method by which wires of great strength are also obtained, but in which etching off proceeds in a reliable and regular manner.

According to the invention such a method is characterized in that the boron surface is etched off with an etchant containing 55 to 85 percent by weight of  $H_3PO_4$ , 2 to 20 percent by weight of  $HNO_3$  and 10 to 35 % by weight of water.

It was found that optimum results are obtained when the temperature of the etchant is approximately 100°C.

When using the said etchants, the etching rate is at least approximately 2.5 micrometres per minute. The advantage of these etchants as compared with the use of nitric acid as an etchant is that this rate is immediately achieved for all wires and that, consequently, there is no run-in period. This means that after the etching rate of a bath is determined, any desired decrease in diameter may be obtained by etching the wires over a predetermined period.

Etching rates of approximately 4.5 micrometres per minute and more may be obtained with etchants which contain from 70 to 85 percent by weight of  $H_3PO_4$ , 2

to 15 percent by weight of  $HNO_3$  and 10 to 25 percent by weight of water.

In order that the invention may be readily carried into effect, it will now be described with reference to 5 several examples.

**EXAMPLE I**

An etching bath of the following composition was prepared

10 78.1 % by weight of  $H_3PO_4$   
4.9 % by weight of  $HNO_3$   
17.0 % by weight of  $H_2O$   
by mixing 10 parts by volume of concentrated  $HNO_3$  (60 percent by weight of  $HNO_3$  in water) with 90 parts 15 by volume of  $H_3PO_4$  (85 percent by weight of  $H_3PO_4$  in water). The etching rate was determined on wires having a diameter of 96 micrometres which had been obtained as follows:

20 A tungsten wire having a diameter of 12.5 micrometres was passed at a constant rate through a space through which gaseous boron trichloride and hydrogen in a mixture ratio of 1:3 was passed.

The tungsten wire was heated by a direct current passage at a temperature of approximately 1,100°C.

25 The etching-off rates were determined by etching wire pieces with the etchant (temperature 100°C).

The results mentioned in Table I were obtained.

**TABLE I**

| 30<br>etching time<br>in minutes | Wire diameter                     |                                | etching rate<br>in $\mu m$ per min. |
|----------------------------------|-----------------------------------|--------------------------------|-------------------------------------|
|                                  | prior to<br>etching<br>in $\mu m$ | after<br>etching<br>in $\mu m$ |                                     |
| 35                               | 1                                 | 96                             | 83                                  |
|                                  | 2                                 | 96                             | 75                                  |
|                                  | 3                                 | 96                             | 65.5                                |
|                                  | 4                                 | 96                             | 57.5                                |
|                                  | 5                                 | 96                             | 51.5                                |

**EXAMPLE II**

As in Example I, 5 wires having a diameter of 97  $\mu m$  were etched for one minute. The average tensile strength prior to etching was 229 kg/sq.mm, after etching it was 297 kg/sq.mm, which is an increase of the average tensile strength by approximately 30 percent.

**EXAMPLE III**

An etchant having the following composition was prepared:

66.3 % by weight of  $H_3PO_4$   
5.3 % by weight of  $HNO_3$   
28.4 % by weight of  $H_2O$   
by mixing 70 parts by volume of  $H_3PO_4$  (85 %), 10 parts by volume of  $HNO_3$  (60 %) and 20 parts by volume of water.

55 Wires (diameter 90  $\mu m$ ) were etched for 5 minutes with this etchant (temperature 100°C) and the average etching rate was 2.9 micrometres per minute.

**EXAMPLE IV**

The etchant according to Example I was compared with an etchant consisting of 42.5 percent by weight of  $HNO_3$  obtained by mixing 64 parts by volume of concentrated  $HNO_3$  with 36 parts by volume of water. Then the results according to Table II were obtained:

TABLE II

| etching<br>time in<br>minutes | Etchant according to<br>Example I                |                                  |     | 42.5% by weight of HNO <sub>3</sub> aq          |                                     |     |
|-------------------------------|--------------------------------------------------|----------------------------------|-----|-------------------------------------------------|-------------------------------------|-----|
|                               | diameter<br>after<br>etching<br>in $\mu\text{m}$ | tensile<br>strength<br>kg/sq.mm. |     | diameter<br>after et-<br>ching in $\mu\text{m}$ | tensile<br>strength in<br>kg/sq.mm. |     |
|                               |                                                  | A                                | B   |                                                 | A                                   | B   |
| 0                             | 96                                               | 301                              | 291 | 96                                              | 301                                 | 291 |
| 1                             | 83                                               | 316                              | 342 | 90                                              | 308                                 | 304 |
| 2                             | 73                                               | 336                              | 294 | 85                                              | 305                                 | 287 |
| 3                             | 65                                               | 320                              | 308 | 80                                              | 293                                 | 281 |
| 4                             | 57                                               | 241                              | 229 | 62                                              | 233                                 | 241 |
| 5                             | 50                                               | 190                              | 202 | 55                                              | 101                                 | 98  |

A = tensile length 10 cm.

B = tensile length 1 cm.

Table II shows that with the etchant according to Example I, starting from the same average tensile strength level prior to etching for a comparable decrease in diameter, always higher values of the average tensile strength are obtained than with an etchant comprising nitric acid only.

What is claimed is:

1. A method of improving the physical properties of a boron wire produced by deposition of a gaseous mixture comprising a volatile boron compound on a hot substrate comprising, etching the resultant boron surface with an etchant comprising 55 to 85 percent by weight of H<sub>3</sub>PO<sub>4</sub>, 2 to 20 percent by weight of HNO<sub>3</sub>

and 10 to 35 percent by weight of water at a rate of at least about 2.5 micrometres per minute and at a temperature sufficiently high to remove surface errors from the boron surface.

2. A method as claimed in claim 1, characterized in that the etchant is used at a temperature of approximately 100°C.

3. A method as claimed in claim 1, characterized in that the boron surface is etched off with an etchant comprising 70 to 85 percent by weight of H<sub>3</sub>PO<sub>4</sub>, 2 to 15 percent by weight of HNO<sub>3</sub> and 10 to 25 percent by weight of water.

\* \* \* \* \*

35

40

45

50

55

60

65